

## UNITED STATES PATENT OFFICE.

JEREMIAH BUTLER, OF OXFORD, PENNSYLVANIA, ASSIGNOR OF ONE-HALF TO ISAAC P. WALTON, OF OXFORD, PENNSYLVANIA.

## SOLDER FOR ALUMINUM.

No Drawing.

Application filed December 30, 1927. Serial No. 243,772.

The present invention relates to an improved solder for various metals and particularly for aluminum. It is the purpose of the present invention 5 to compound a composition of matter constituting a very effective solder, one capable of adjoining opposing pieces of metal, namely aluminum, making a joint very lasting as well as efficient, capable of withstanding 10 heavy strains.

It is to be understood that the particulars herein given are in no way limitive, and that while still keeping within the scope of the invention, any desired modification of 15 details and proportions may be made in the composition of matter according to circumstances.

The invention comprises further features and combination of ingredients to be hereinafter set forth and claimed.

The herein specified composition of matter consists of using a steel or cast iron vessel having a large surface bottom, in which requisite amount of steel filings are deposited, 25 sufficient heat being applied to bring the filings to a red heat, a quantity of block tin, steel, borax, plaster of Paris, with salt, all of which is ground or reduced to a fine state, the composition of matter consisting of the block 30 tin, steel, borax, plaster of Paris, and salt being deposited in the molten metal, reduced from the steel filings, reserving one-third of such composition of block tin, steel, borax, plaster of Paris and salt to be applied to the 35 matter within five minutes of the time of

pouring the composition matter in a mold, which is kept continually hot to a red heat for at least forty-five minutes, with silver added in the last five minutes while in a molten state.

In order to compound a quantity of twenty-five pounds the foregoing ingredients are compounded in the following proportions, to wit:

|                  |       |     |    |
|------------------|-------|-----|----|
| Steel filings    | 1     | lb. | 45 |
| Block tin        | 25    | lb. |    |
| Steel            | 1/2   | oz. |    |
| Borax            | 3 1/2 | oz. |    |
| Plaster of Paris | 4     | oz. | 50 |
| Salt             | 1     | lb. |    |
| Silver           | 12    | oz. |    |

While these proportions are herein named for making twenty-five pounds of solder for aluminum, it is obvious that to compound a greater quantity or a less quantity the various ingredients may be proportionately increased or decreased.

The invention having been set forth, what is claimed is:

A composition of soldering matter for aluminum consisting of steel filings one pound, block tin twenty-five pounds, steel one-half ounce, borax three and one-half ounces, plaster of Paris four ounces, salt one pound, and twelve ounces of silver.

In testimony whereof he affixes his signature.

JEREMIAH BUTLER.